



US005387559A

**United States Patent** [19]

Nagata et al.

[11] **Patent Number:** **5,387,559**[45] **Date of Patent:** **Feb. 7, 1995****[54] RESISTIVE PASTE**

[75] Inventors: **Keisuke Nagata; Hiroji Tani**, both of Kyoto, Japan

[73] Assignee: **Murata Manufacturing Co., Ltd.**, Kyoto, Japan

[21] Appl. No.: **68,959**

[22] Filed: **May 28, 1993**

**[30] Foreign Application Priority Data**

May 28, 1992 [JP] Japan ..... 4-136888

[51] Int. Cl.<sup>6</sup> ..... **H01C 7/00**

[52] U.S. Cl. ..... **501/20; 501/17;**  
501/18; 501/96; 501/98; 232/521; 232/518

[58] **Field of Search** ..... 252/518, 521; 501/17,  
501/18, 20, 96, 98

**[56] References Cited****U.S. PATENT DOCUMENTS**

5,036,027 7/1991 Watanabe et al. ..... 501/96  
5,196,915 3/1993 Ho et al. ..... 252/318

**FOREIGN PATENT DOCUMENTS**

8133 2/1980 European Pat. Off. ..... 252/321

*Primary Examiner*—Mark L. Bell

*Assistant Examiner*—C. M. Bonner

*Attorney, Agent, or Firm*—Ostrolenk, Faber, Gerb & Soffen

**[57] ABSTRACT**

A resistive paste comprising (a) a mixture of a resistive material having a composition of  $Nb_xLa_{1-x}B_{6-4x}$ , wherein x is from 0.1 to 0.9 mol, and non-reducing glass frit, (b) at least one additive selected from the group consisting of  $Li_2O$ ,  $MgO$ ,  $CaO$ ,  $TiO_2$ ,  $MnO_2$ ,  $CuO$ ,  $SrO$ ,  $BaO$ , and  $La_2O_3$  in an amount of from 1 to 10% by weight based on the mixture (a), and (c) an organic vehicle. The resistive paste provides a resistor having its temperature coefficient of resistivity shifted to the minus (—) direction according to necessity.

**14 Claims, No Drawings**

## RESISTIVE PASTE

## FIELD OF THE INVENTION

The present invention relates to a resistive paste which can be baked in a neutral or reducing atmosphere.

## BACKGROUND OF THE INVENTION

A circuit pattern, which is composed of electrodes on which various electronic parts are mounted and resistors, has been generally formed on a ceramic base made of alumina, zirconia, etc., and the electrodes are generally formed by screen printing a conductive paste containing a noble metal, e.g., Ag or Ag-Pd, on the ceramic base followed by baking in air. Because of its cost, the noble metallic paste has recently been displaced with a conductive paste containing a base metal, e.g., Cu, Ni or Al. In using such a base metallic paste, the screen-printed paste on a ceramic base is generally baked in a neutral or reducing atmosphere. If the base metallic paste is heated at high temperatures (i.e., baked) in an oxygen-containing atmosphere, such as air, a metal oxide which is an insulator would be formed. This is the reason why baking of a base metallic paste should be conducted in a neutral or reducing atmosphere.

When electrodes are formed by using such a base metallic paste, resistors which are arranged to bridge over the electrodes should also be formed by using a resistive paste which can be baked in a neutral or reducing atmosphere. Known resistive pastes which can be baked in a neutral or reducing atmosphere include LaB<sub>6</sub>-based pastes, NbB<sub>2</sub>-based pastes, and the resistive paste proposed by the present inventors and disclosed in U.S. Pat. No. 5,036,027. The paste described in U.S. Pat. No. 5,036,027 comprises a mixture of a resistive material having a composition of Nb<sub>x</sub>La<sub>1-x</sub>B<sub>6-4x</sub> (wherein x is from 0.1 to 0.9 mol) and non-reducing glass frit, kneaded with an organic vehicle.

A desired surface resistivity over a broad range has been obtained by varying the mixing ratio of these resistive materials and glass frit. However, in using the LaB<sub>6</sub>-based or NbB<sub>2</sub>-based resistive pastes, the surface resistivity suffers drastic changes with a slight variation in glass frit amount, and satisfactory reproducibility cannot be assured. On the other hand, resistors formed of the Nb<sub>x</sub>La<sub>1-x</sub>B<sub>6-4x</sub>-based paste show a milder increase in surface resistivity than with those formed of the LaB<sub>6</sub>-based pastes and NbB<sub>2</sub>-based pastes. Therefore, the Nb<sub>x</sub>La<sub>1-x</sub>B<sub>6-4x</sub>-based paste has an advantage of a broadened surface resistivity range of from 10 Ω/square to 10 MΩ/square by varying the mixing ratio of resistive material to glass frit. However, the resistors formed of the Nb<sub>x</sub>La<sub>1-x</sub>B<sub>6-4x</sub>-based paste, particularly those adjusted to have a low surface resistivity (e.g., from 10 Ω/square to 3 kΩ/square), sometimes undergo deterioration in their temperature coefficient of resistivity (hereinafter abbreviated as "TCR"), i.e., a shift of TCR in the plus (+) direction, and do not always satisfy the characteristics required for practical use.

## SUMMARY OF THE INVENTION

An object of the present invention is to provide a resistive paste which can be baked in a neutral or reducing atmosphere and whose TCR can be shifted to the minus (-) direction according to necessity.

Other objects and effects of the present invention will be apparent from the following description.

The present invention provides a resistive paste comprising (a) a mixture of a resistive material having a composition of Nb<sub>x</sub>La<sub>1-x</sub>B<sub>6-4x</sub>, wherein x is from 0.1 to 0.9 mol, and non-reducing glass frit, (b) at least one additive selected from the group consisting of Li<sub>2</sub>O, MgO, CaO, TiO<sub>2</sub>, MnO<sub>2</sub>, CuO, SrO, BaO, and La<sub>2</sub>O<sub>3</sub> in an amount of from 1 to 10% by weight based on the mixture (a), and (c) an organic vehicle.

## DETAILED DESCRIPTION OF THE INVENTION

In the present invention, Nb<sub>x</sub>La<sub>1-x</sub>B<sub>6-4x</sub>, wherein x is from 0.1 to 0.9 mol, preferably from 0.2 to 0.8 mol, is used as a resistive material. If x is less than 0.1 mol, it tends to be difficult to gradually increase the surface resistivity, while if x is more than 0.9 mol, the change rate of surface resistivity with the content of glass frit tends to become large, thus making it difficult to improve the reproducibility of the surface resistivity.

The grain size of the resistive material is generally from 0.1 to 5 μm. If the grain size is less than 0.1 μm, a prolonged period of grinding time is required to prepare the resistive material, and impurities introduced during the grinding tend to adversely affect the properties of the resistive material. If the grain size is more than 5 μm, it tends to be difficult to obtain a constant resistivity in a stable manner.

30 The resistive material can be prepared in any conventional manners, such as those described in U.S. Pat. No. 5,036,027.

Examples of the non-reduced glass frit used in the present invention include alkali earth boroaluminosilicate, etc. The grain size of the non-reduced glass frit is generally from 1 to 10 μm. If the grain size is less than 1 μm, the change rate of surface resistivity tends to be too large, while if it is more than 10 μm, it tends to be difficult to obtain uniform resistors in a stable manner. The non-reduced glass frit can be prepared in any conventional manner, such as by mixing appropriate oxides followed by being fused.

The weight ratio of the resistive material to the non-reduced glass frit can be widely varied depending on 45 the desired surface resistivity and the like, and is generally from 5/100 to 70/100 by weight in the present invention.

At least one additive selected from the group consisting of Li<sub>2</sub>O, MgO, CaO, TiO<sub>2</sub>, MnO<sub>2</sub>, CuO, SrO, BaO, and La<sub>2</sub>O<sub>3</sub> is added to the mixture of resistive material and glass frit in an amount of from 1 to 10% by weight, preferably from 2 to 8% by weight, based on the mixture. If it is less than 1% by weight, the effect of the additive would not be obtained, while if it is more than 10% by weight, the TCR becomes too large. The grain size of the additive is generally from 0.5 to 5 μm. If the grain size is outside this range, the effect of the additive tends to be insufficient, resulting in deterioration of the resulting resistor.

60 An organic vehicle is used for forming the resistive paste according to the present invention. Examples thereof include an acrylic resin and an ethylcellulose diluted with terpenes such as α-terpineol, β-terpineol or a mixture thereof with other solvents such as kerosine, butyl carbitol, butyl carbitol acetate and high boiling alcohols and alcohol esters. The organic vehicle should be thixotropic in order that it set up rapidly after being screened, thereby giving good resolution.

The resistive paste of the present invention can be produced in any conventional manner for preparing resistive pastes. For example, a resistive material and a glass frit, which have been separately prepared, are mixed with an additive, and the resulting mixture is kneaded with an organic vehicle to form a resistive paste according to the present invention.

The resistive paste of the present invention can be used in a manner similar to conventional resistive pastes. For example, the resistive paste can be printed 10 on a suitable base, such as a ceramic base, by screen printing, dried at 150° C. for 10 minutes, and then baked at a peak temperature at 900° C. for 10 minutes in a nitrogen atmosphere.

The surface resistivity of the resistor, which is formed 15 from the resistive paste of the present invention, is not particularly limited and is generally from 10 Ω/square to 10 kΩ/square, and preferably from 20 Ω/square to 5 kΩ/square.

The present invention will be illustrated in greater 20 detail with reference to Example, but it should be understood that the present invention is not construed as being limited thereto. All the percents are by weight unless otherwise indicated.

### EXAMPLE

#### Preparation of Electrodes

A conductive paste containing Cu as a base metal was screen printed on an alumina ceramic base and baked in 30 a nitrogen atmosphere to form electrodes.

#### Preparation of Resistive Paste

Powdered NbB<sub>2</sub> and LaB<sub>6</sub> were weighed and mixed to provide a composition of Nb<sub>x</sub>La<sub>1-x</sub>B<sub>6-4x</sub>, with x being varied between 0.1 mol and 0.9 mol as shown in Table 1 below. The mixture was calcined in a nitrogen atmosphere for 2 hours at a temperature increase rate of 3° C./min with the peak temperature set at 1000° C. to prepare a solid solution of LaB<sub>6</sub> in NbB<sub>2</sub>. The resulting mixture was ground in a vibration mill to an average particle size of 1 μm and dried to obtain a resistive material having a composition of Nb<sub>x</sub>La<sub>1-x</sub>B<sub>6-4x</sub> (where x is 0.1 to 0.9 mol).

Separately, B<sub>2</sub>O<sub>3</sub>, SiO<sub>2</sub>, BaO, CaO, Nb<sub>2</sub>O<sub>5</sub>, and K<sub>2</sub>O 45 were mixed at a molar ratio of 35.56/31.24/17.78/10.04/2.41/2.97 and fused at a temperature of from 1,200° to 1,350° C. to prepare fused glass. The fused glass was quenched in pure water and ground in a vibration mill to an average particle size of 50 5 μm or smaller to prepare non-reducing glass frit.

Li<sub>2</sub>O, MgO, CaO, TiO<sub>2</sub>, MnO<sub>2</sub>, CuO, SrO, BaO or La<sub>2</sub>O<sub>3</sub> was added to a mixture composed of 40% by weight of the resistive material and 60% by weight of the non-reducing glass frit in an amount varying from 0 55 to 12% based on the mixture as shown in Table 1.

The resulting mixture was kneaded with an organic vehicle composed of an acrylic resin diluted with α-terpineol to prepare a resistive paste.

TABLE 1

| Sample No. | x (mol) | Resistive material (wt %) | Glass frit (wt %) | Kind and amount of additive (wt %**) | 60 |
|------------|---------|---------------------------|-------------------|--------------------------------------|----|
| 1*         | 0.25    | 40                        | 60                | none                                 | 0  |
| 2          | 0.25    | 40                        | 60                | TiO <sub>2</sub>                     | 3  |
| 3          | 0.25    | 40                        | 60                | TiO <sub>2</sub>                     | 7  |
| 4*         | 0.25    | 40                        | 60                | TiO <sub>2</sub>                     | 12 |
| 5          | 0.25    | 40                        | 60                | MgO                                  | 3  |

TABLE 1-continued

| Sample No. | x (mol) | Resistive material (wt %) | Glass frit (wt %) | Kind and amount of additive (wt %**) |    |
|------------|---------|---------------------------|-------------------|--------------------------------------|----|
| 6          | 0.25    | 40                        | 60                | MgO                                  | 7  |
| 7          | 0.25    | 40                        | 60                | La <sub>2</sub> O <sub>3</sub>       | 3  |
| 8          | 0.25    | 40                        | 60                | Li <sub>2</sub> O                    | 3  |
| 9          | 0.25    | 40                        | 60                | CaO                                  | 3  |
| 10         | 0.25    | 40                        | 60                | MnO <sub>2</sub>                     | 3  |
| 11         | 0.25    | 40                        | 60                | CuO                                  | 7  |
| 12         | 0.25    | 40                        | 60                | SrO                                  | 7  |
| 13         | 0.25    | 40                        | 60                | BaO                                  | 7  |
| 14*        | 0.75    | 40                        | 60                | none                                 | 0  |
| 15         | 0.75    | 40                        | 60                | TiO <sub>2</sub>                     | 3  |
| 16         | 0.75    | 40                        | 60                | TiO <sub>2</sub>                     | 7  |
| 17*        | 0.75    | 40                        | 60                | TiO <sub>2</sub>                     | 12 |
| 18         | 0.75    | 40                        | 60                | MgO                                  | 3  |
| 19         | 0.75    | 40                        | 60                | MgO                                  | 7  |
| 20         | 0.75    | 40                        | 60                | La <sub>2</sub> O <sub>3</sub>       | 3  |
| 21         | 0.75    | 40                        | 60                | Li <sub>2</sub> O                    | 3  |
| 22         | 0.75    | 40                        | 60                | CaO                                  | 3  |
| 23         | 0.75    | 40                        | 60                | MnO <sub>2</sub>                     | 3  |
| 24         | 0.75    | 40                        | 60                | CuO                                  | 7  |
| 25         | 0.75    | 40                        | 60                | SrO                                  | 7  |
| 26         | 0.75    | 40                        | 60                | BaO                                  | 7  |

Note:

\*Samples out of the scope of the present invention.

\*\*Based on the mixture of resistive material and glass frit.

#### Preparation of Resistor

Each of the resistive pastes was screen printed on the 30 ceramic base in a size of 1.5 mm long and 1.5 mm wide including a part of electrode between electrodes, dried at 150° C. for 10 minutes, and baked in a nitrogen atmosphere with the peak temperature set at 900° C. for 10 minutes to form a resistor.

#### Evaluation

The surface resistivity and TCR of each sample thus prepared were measured. The results obtained are shown in Table 2 below.

TABLE 2

| Sample No. | Surface Resistivity (Ω/square) | TCR (ppm/°C.) |         |
|------------|--------------------------------|---------------|---------|
|            |                                | +150° C.      | -55° C. |
| 1*         | 79                             | +725          | +670    |
| 2          | 66                             | +410          | +370    |
| 3          | 59                             | +210          | +175    |
| 4*         | 537                            | +630          | +580    |
| 5          | 70                             | +510          | +485    |
| 6          | 67                             | +325          | +270    |
| 7          | 77                             | +390          | +370    |
| 8          | 93                             | +435          | +380    |
| 9          | 72                             | +660          | +620    |
| 10         | 83                             | +645          | +610    |
| 11         | 107                            | +410          | +360    |
| 12         | 75                             | +585          | +545    |
| 13         | 61                             | +490          | +450    |
| 14*        | 3,140                          | +430          | +390    |
| 15         | 2,300                          | +150          | +390    |
| 16         | 1,910                          | +15           | -35     |
| 17*        | 9,850                          | +415          | +370    |
| 18         | 2,700                          | +240          | +195    |
| 19         | 2,200                          | +115          | +75     |
| 20         | 2,920                          | +95           | +110    |
| 21         | 4,320                          | +315          | +260    |
| 22         | 2,890                          | +380          | +345    |
| 23         | 3,300                          | +375          | +335    |
| 24         | 4,530                          | +200          | +170    |
| 25         | 2,950                          | +315          | +265    |
| 26         | 2,330                          | +270          | +235    |

It can be seen from Table 2 that Sample No. 1 containing no additive in accordance with the conventional

technique ( $x=0.75$  mol) had TCR of +725 ppm/ $^{\circ}$  C. and +670 ppm/ $^{\circ}$  C. and similarly Sample No. 14 ( $x=0.75$  mol) had TCR of +430 ppm/ $^{\circ}$  C. and +390 ppm/ $^{\circ}$  C., while samples containing 1 to 10% of the additive according to the present invention (Sample Nos. 2, 3 and 5 to 13 and Sample Nos. 15, 16 and 18 to 26) had their TCR shifted to the minus (–) direction as compared with Sample No. 1 or No. 14. It is also apparent that Sample Nos. 4 and 17 containing more than 10% of the additive show little improvement in TCR.

As described and demonstrated above, the resistive paste according to the present invention comprises a mixture of a resistive material having a composition of  $Nb_xLa_{1-x}B_{6-4x}$  ( $x=0.1$  to  $0.9$  mol) and non-reducing glass frit and further contains at least one additive selected from the group consisting of  $Li_2O$ ,  $MgO$ ,  $CaO$ ,  $TiO_2$ ,  $MnO_2$ ,  $CuO$ ,  $SrO$ ,  $BaO$ , and  $La_2O_3$  in an amount of from 1 to 10% by weight based on the mixture. According to the present invention, it is possible to shift the temperature coefficient of surface resistivity of a resistor formed by baking an  $Nb_xLa_{1-x}B_{6-4x}$ -based resistive paste particularly in a low resistivity range to the minus (–) direction so that the resistive paste of the present invention sufficiently satisfies the characteristics required for a resistive paste to be based in a neutral or reducing atmosphere.

While the invention has been described in detail and with reference to specific examples thereof, it will be apparent to one skilled in the art that various changes and modifications can be made therein without departing from the spirit and scope thereof.

What is claimed is:

1. In a resistive paste comprising (a) a mixture of a resistive material having a composition of  $Nb_xLa_{1-x}B_{6-4x}$ , wherein  $x$  is from 0.1 to 0.9 mol, and non-reducing glass frit and (b) an organic vehicle, the improvement which comprises the presence of (c) at least one addi-

tive selected from the group consisting of  $Li_2O$ ,  $MgO$ ,  $CaO$ ,  $TiO_2$ ,  $MnO_2$ ,  $CuO$ ,  $SrO$  and  $BaO$  in an amount of from 1 to 10% by weight based on said mixture (a), whereby the temperature coefficient of resistivity is shifted in the minus direction by the presence of additive (c).

2. The resistive paste of claim 1 in which the additive amount is 2 to 8%.

3. The resistive paste of claim 2 in which the additive has a particle size of 0.5 to 5  $\mu$ m.

4. The resistive paste of claim 3 in which the particle size of the resistive material is from 0.5 to 5  $\mu$ m and the particle size of the glass frit is from 1 to 10  $\mu$ m.

5. The resistive paste of claim 4 in which the weight ratio of the resistive material to glass frit is from 5/100 to 70/100 by weight.

6. The resistive paste of claim 1 in which the additive is  $Li_2O$ .

7. The resistive paste of claim 1 in which the additive is  $MgO$ .

8. The resistive paste of claim 1 in which the additive is  $CaO$ .

9. The resistive paste of claim 1 in which the additive is  $TiO_2$ .

10. The resistive paste of claim 1 in which the additive is  $MnO_2$ .

11. The resistive paste of claim 1 in which the additive is  $CuO$ .

12. The resistive paste of claim 1 in which the additive is  $SrO$ .

13. The resistive paste of claim 11 in which the additive is  $BaO$ .

14. The resistive paste of claim 1 in which the baked paste has a surface resistivity of from 10 to 3,0000 ohms per square.

\* \* \* \* \*